

Nov. 21, 1933.

F. MAULEN

1,936,333

PIN FOR ARTIFICIAL TEETH

Filed May 13, 1932

*Fig. 1*



*Fig. 2*



*Fig. 3*



*Fig. 4*



*Fig. 5*



INVENTOR.  
*Frederick Maulen*,  
BY  
*Wenett & Kook*,  
ATTORNEYS.

## UNITED STATES PATENT OFFICE

1,936,333

## PIN FOR ARTIFICIAL TEETH

Frederick Maulen, East Orange, N. J., assignor  
to Baker & Company, Inc., Newark, N. J., a  
corporation of New Jersey

Application May 13, 1932. Serial No. 611,019

4 Claims. (Cl. 32—9)

This invention relates to pins for artificial teeth, i. e., pins that are secured in the lingual sides of artificial teeth for attaching the teeth to backings.

- 5 Such pins usually include a body or core of a strong relatively inexpensive metal which will withstand soldering and the strains imposed on an artificial tooth, for example, nickel or an alloy. It is impracticable to use a pin formed wholly of such metals because these metals easily and quickly oxidize or corrode, especially under the action of fluids in the mouth, which might render soldering difficult if not impossible and cause loosening of the pin in a tooth or a backing. 10 Therefore it has been the practice to coat the body or core with a layer of substantially non-corrosive metal of considerable thickness which will also withstand soldering temperatures, such coating protecting the body of the pin from the corrosive action of fluids in the mouth. Gold is generally used for this coating, but the coating must be so thick to prevent corrosion as to make the pin quite expensive. Gold is not sufficiently strong for use alone in such pins, and especially 15 is too expensive; in fact gold is so expensive that probably it would not be used at all for the purpose if a corrosion-resisting coating were not required on the nickel body of the pins.

One object of my invention is to provide a 20 tooth pin of the general character described embodying novel and improved features of construction which shall have the equivalent or superior corrosion-resisting qualities and strength and at the same time shall be considerably less expensive than the known pins.

Another object is to provide such a tooth pin having a core or body of nickel or other suitable inexpensive metal, and one or more coatings or layers of precious metals or alloys thereof which 25 will resist corrosion under influence of oral fluids, withstand soldering temperatures and are less expensive than gold, said layers being coated with an outside layer of gold, whereby it shall be possible to use a thinner layer of gold than has been used heretofore and to provide a pin 30 having corrosion-resisting qualities equivalent or superior to those of known pins, and at less cost.

Other objects of my invention are to provide a tooth pin having a core of nickel or other suitable metal, and a plurality of coating layers of non-corrosive or corrosion-resisting precious metals the corrosion-resisting qualities of which are successively greater from the inner layer to the outer layer.

55 I have found that palladium, and certain alloys

of palladium, for example palladium and gold, palladium and silver, palladium, gold and silver, and even silver alone where the soldering temperatures are low, may be used to form the layer or layers between the core and the outer layer 60 of gold. These metals and alloys are less expensive than gold and they serve as a buffer between the easily oxidizable surface of the core and the outer layer of gold which accordingly may be very thin or skin-like.

Therefore other objects of the invention are to provide a tooth pin comprising a core of nickel or other suitable metal having a coating of one or more inner layers of palladium or certain alloys thereof with other metals, or a layer of 70 silver, and a thin outer layer of gold; and to obtain other advantages and results as will be brought out by the following description.

Referring to the accompanying drawing, in which corresponding and like parts are designated 75 throughout the several views by the same reference characters,

Figure 1 is a transverse vertical sectional view through an artificial tooth facing, showing a tooth pin embodying my invention therein; 80

Figure 2 is an elevation of the lingual side of the tooth showing the pins in end elevation;

Figure 3 is an enlarged sectional elevation of one of the pins;

Figure 4 is a sectional elevation through a 85 piece of wire from which the pin is formed, and

Figure 5 is a transverse vertical sectional view, on the line 5—5 of Figure 3.

Specifically describing the illustrated embodiment of the invention, the reference character A 90 designates a porcelain tooth of known construction, and B designates a pin embodying my invention which is secured at one end in an anchor ring C which is embedded in the tooth. The outer extremity of the pin has a head D as usual 95 for attaching the pin to a tooth backing.

Such pins are usually made of lengths of wire, the heads D being formed by swaging or upsetting one end of the wire. It is necessary that the exterior surface of the pin be substantially 100 non-corrosive or corrosion-resisting and it is also necessary that the pin be formed of such metal as will provide the necessary strength and withstand the usual soldering temperatures; and, of course, it is desirable that the pins be as inexpensive as possible. Accordingly, pins of this character are usually formed with a body or core 1 of a suitable relatively inexpensive base metal, for example nickel, and because the base metal easily and quickly corrodes, especially under the 110

destructive action of acids in the mouth, it is the general practice to coat the core with a non-corrosive or corrosion-resisting layer, which is usually gold. It is necessary that this corrosion-resisting layer be of considerable thickness in order to adequately protect the core from corrosion, and when the layer is made of gold, the pin is expensive. It will be understood by those skilled in the art that the coating layer may be applied in any suitable manner.

In accordance with the invention, the core 1 is provided with a plurality of coating layers of different corrosion-resisting metals which will also withstand soldering temperatures, and preferably the outer layer is of gold and the inner layers are of some less expensive precious metals. The inner layers may be for example palladium, or an alloy of palladium and gold, or an alloy of palladium and silver, or an alloy of palladium, gold and silver, and may even be silver alone where the soldering temperatures are low. Obviously, other suitable corrosion-resisting metals may be used instead of palladium or silver, or alloys of palladium or silver with other metals.

In the drawing, the reference character 2 designates an inner layer of corrosion-resisting metal, for example palladium, and 3 designates the outer layer of corrosion-resisting metal. The inner layer may be thicker than the outer layer, and therefore the outer layer may be thinner than the coating layer of gold which has been used heretofore in such tooth pins, the inner layer serving as a buffer between the core and the outer layer which is usually gold.

In accordance with the invention, the metal of the inner layer 2 may have a corrosion-resisting quality less than that of gold, and the thickness thereof may be varied as required to provide the desirable corrosion-resisting effect. Also, obviously the number of layers or coatings may be varied as desired, and while it is desirable that gold be the outer layer, such is not necessary to the provision of a satisfactory tooth pin.

From the foregoing, it will be understood that with my invention a non-corrosive wire is provided, particularly for use in making pins for artificial teeth, which has corrosion-resisting qualities and strength equal or superior to the respec-

tive corrosion-resisting qualities and strength of known pins or non-corrosive wire, and at less cost, and the external appearance of the wire of the pins may be identical with that of the highly desirable rich color of known gold covered wire or pins.

With my invention I can make the gold outer coating very thin and utilize a heavier buffer coating of palladium, or the like, which, particularly because palladium is less expensive and has a lower specific gravity than gold, enables me to provide a pin or wire equivalent or superior to known gold covered pins or wire at much less cost.

Various modifications in the relative arrangement of the layers of corrosion-resisting metals, and various other metals than those mentioned, may be utilized without departing from the spirit or scope of the invention, and therefore I do not desire to be understood as limiting myself in the construction and use of the invention except as required by the following claims when construed in the light of the prior art.

The term "precious metal" as used in this specification and the appended claims is intended to include all of the precious metals and precious metal alloys hereinbefore set forth and their equivalents for the purpose specified. The term "corrosion resisting" means capable of resisting corrosion or susceptible to negligible corrosion, under the action of oral fluids.

Having thus described the invention, what I claim is:

1. A tooth pin comprising a core of metal having a plurality of coating layers of different corrosion-resisting precious metals.

2. A tooth pin comprising a core of metal having an outer thin coating layer of gold, and a coating layer of different corrosion-resisting precious metal between said layer of gold and said core.

3. A tooth pin comprising a core of metal having an inner coating layer of palladium, and an outer coating layer of gold.

4. A tooth pin comprising a core of metal having an inner coating layer of silver and an outer coating layer of gold.

FREDERICK MAULEN.